

1,312,480.

S. HULDT,  
METHOD OF REFINING ZINC,  
APPLICATION FILED APR. 3, 1917.

Patented Aug. 5, 1919.



Fig. 1.



Fig. 2.



Fig. 3



Fig. 4.

WITNESS.

H. Crawford.

INVENTOR.

SVEN HULDT

BY A. E. Parker

ATTORNEY.

# UNITED STATES PATENT OFFICE.

SVEN HULDT, OF STOCKHOLM, SWEDEN, ASSIGNOR TO NORSK ELEKTRISK METALINDUSTRI AKTIESELSKAP, OF SUNDLÖKKEN, SARPSBORG, NORWAY.

## METHOD OF REFINING ZINC.

1,312,480.

Specification of Letters Patent.

Patented Aug. 5, 1919.

Application filed April 3, 1917. Serial No. 159,508.

To all whom it may concern:

Be it known that I, SVEN HULDT, residing at Stockholm, Sweden, have invented certain new and useful Improvements in 5 Methods of Refining Zinc, of which the following is a specification.

The present invention has for its object to provide an improved method of refining zinc, whereby refined zinc of the desired 10 degree of purity is obtained with economy in heat and in a continuous manner.

The refining operation according to the present invention is carried out continuously, by the employment of radiant heat produced 15 by electrical means and by employing special means for obtaining zinc of great purity, uniformity in operation of the refining process and economy in the amount of current consumed.

20 In the accompanying drawing Figure 1 is a transverse section and Fig. 2 a longitudinal section of a furnace for refining zinc according to the present invention, proportioned as above described. The zinc to be refined is assumed to contain 0.5% of lead, and the bath surface is given the size of 0.5 square meters. 1 indicates the furnace, and 2 the electrodes projecting through openings in the furnace walls, and establishing an arc 25 for heating the zinc bath contained in the furnace. 3 indicates a receiver in communication with the furnace chamber at the bottom thereof, and serving as a sealed inlet, through which the zinc to be refined is fed 30 into the furnace chamber. 4 indicates the escape opening for the refined zinc vapors. In this furnace the depth of the zinc bath 5 is 5 centimeters. 6 is a tapping hole for drawing off the lead layer 7, gradually 35 gathering on the bottom of the furnace chamber, so that the superposed layer of zinc 5 will approximately maintain its depth above indicated.

40 Figs. 3 and 4 are views similar to Figs. 1 and 2, illustrating a furnace for refining zinc containing 15% lead. Similar letters refer to corresponding parts. The depth of the zinc bath in this furnace will be 100 centimeters.

45 It will be found by tests, that the escaping zinc vapors contain lead, the feed of raw material should be augmented so as to establish a thicker layer of zinc.

50 Obviously the drawing off of lead will be done without interfering with the process of

refining, the heating being continuous, to effect continuous distillation.

Hitherto it has been assumed, that when refining zinc the source of heat will be most economically utilized, if the depth of the 60 molten zinc bath, from the surface of which the zinc is vaporized, is reduced as much as possible. For this purpose it has been proposed according to one known process of refining, to cause the molten zinc to flow in a 65 thin layer from a superposed receiver along an inclined plane, heating said layer during its flow so as to vaporize the zinc.

The present invention however, which is based on extensive investigations and experiments in connection with the refining of zinc in electric radiating furnaces, consists in carrying out the refining operation by employing a molten mass of zinc, which is proportioned and calculated sufficiently 75 great, that the same constitutes a heat magazine or accumulator, sufficiently large to counterbalance considerable variations of temperature. It has been found, that the zinc bath in ordinary processes of refining 80 zinc is subject to considerable variations of temperature, which have an unfavorable influence upon the uniformity of the refining operation, whereas on the other hand such uniformity is a main condition for obtaining 85 a homogeneous and pure product, and sufficient consideration has hitherto not been given to the fact, that the zinc bath, owing to its comparatively small volume, has not been able to counter-balance such variations 90 of temperature.

95 By giving the zinc bath a large volume as above indicated, the advantage is moreover gained, as confirmed by experiments, that the whole process is more economical, owing to the said capability of the zinc bath to accumulate heat, than when a smaller bath is used.

Further, according to the invention, the depth of the zinc bath is proportioned in 100 relation to its surface in such a manner, that lead which is always contained in the material to be refined, is prevented from being distilled during the refining operation. Said depth is proportioned relatively to the furnace capacity by experimentally employing several zinc baths of different depths and testing the zinc distilled from such baths. If the zinc vapors thus distilled contain lead, the depth of the zinc bath employed is too 105 110

small and should be augmented by augmenting the feed of raw material, until lead is no longer present in the vapors. This is a criterion of the fact, that the layer of lead deposited on the bottom of the furnace, underneath the zinc layer is not heated by the superposed zinc layer to the temperature of distillation.

By the term "depth of the bath" above used is understood the depth of the bath at the shallowest place, if the bottom of the furnace is inclined, as toward a tapping place.

By means of the process above described 15 zinc practically free from lead and other impurities, having a purity of 99.9%, may be obtained.

As an example of the proportions above referred to, it may be mentioned that for 20 refining impure zinc containing 0.5 to 15% of lead, the bath surface may be a given size of 0.5 to 9 square meters and the depth of the zinc bath may be from 5 to 100 centimeters.

Having now fully described my invention 25 what I claim is:

1. The method of continuously refining impure zinc by exposing the molten body of

zinc to the action of radiant heat produced by electrical means, which comprises maintaining a body of zinc having such a depth in proportion to the vaporizing surface, that lead from the layer of lead deposited underneath the zinc layer, will remain entirely unvolatilized, whereby pure zinc, free from 35 lead, will volatilize.

2. The method of continuously refining impure zinc by exposing the molten body of zinc to the action of radiant heat produced by electrical means, which comprises 40 maintaining a sufficient depth of the body of zinc in relation to the vaporizing surface, by controlling the feeding of crude zinc, so that the volume of the molten body constitutes a heat magazine adapted to counter-balance variations of temperature created by the source of heat, while distilling off 45 pure zinc from the charge.

In testimony whereof I have signed my name to this specification in the presence of 50 two subscribing witnesses.

SVEN HULDT.

Witnesses:

WAIREMA BOMAN,  
GRETA PRIM.